

1

**3,810,772**  
**FLUOROCHEMICAL COMPOSITIONS FOR**  
**ORGANOPHOBIC SIZING OF PAPER**  
**PRODUCTS**

Melville Willard Uffner, Media, Pa., assignor to Air Products and Chemicals, Inc., Allentown, Pa.  
No Drawing. Continuation-in-part of application Ser. No. 163,417, July 16, 1971, now Patent No. 3,736,164. This application July 21, 1972, Ser. No. 273,980  
Int. Cl. C09k 3/00, 3/18

U.S. Cl. 106—287 R

22 Claims

### ABSTRACT OF THE DISCLOSURE

Improved fluorine-containing phosphate compositions provide enhanced oil and grease resistant properties to cellulosic substrates. Fluorochemicals like polyfluorocycloalkyl phosphates when applied in combination with solvents, surfactants, chelating agents and/or alkali produce a complexing of metallic ions and a wetting effect of cellulosic fibrous bodies thereby enhancing their oleophobic properties. Such compositions are particularly adaptable for economical application to cellulosic stocks which have been previously sized.

### CROSS REFERENCE TO RELATED APPLICATION

This application is a continuation-in-part of application Ser. No. 163,417 filed July 16, 1971, now U.S. Pat. 3,736,164.

### BACKGROUND OF THE INVENTION

The invention relates to functional surface coating compositions having fluorine-containing phosphate materials useful in treating paper and other cellulosic materials for improved oil and grease repellency. Compositions comprising such fluorochemicals in combination with non-fluorinated organic and inorganic wetting or swelling and sequestering agents demonstrate enhanced oleophobic properties when applied to cellulosic materials. They are especially useful for application to paper stock which has been previously sized.

Fluorine-containing monomeric and polymeric materials have been generally acknowledged as useful for application to cellulosic substrates. However, it has been found that certain types of stocks treated with fluorochemical sizing agents perform erratically in terms of imparting oleophobic properties thereto, and accordingly, have not received wide acceptance in industry. More specifically, it has been discovered the performance of fluorochemicals employed in treating paper was unexpectedly diminished on certain base stocks. For example, in the case of rosin/alum sized stock, papers treated with sulphite or in the case of stocks containing lignin and/or groundwood, excessive amounts of fluorochemical sizing were necessary in order to impart satisfactory oleophobic properties.

In many instances, certain cellulosic stocks showed a tendency to preferentially absorb fluorine-containing chemicals disproportionately to the size-tub concentration resulting in pre-mature exhaustion of the size bath, so that pickup at the end of the run was significantly less than experienced at the beginning of the run. Consequently, fluorochemical sizing agents have not received universal acceptance, simply because they were too costly for economical use on all types of stock. That is to say, heretofore, the application of fluorochemical agents has been restricted almost exclusively to waterleaf or unsized stock, and as a result, manufacturers customarily avoided their use on previously sized cellulosics.

2

One remedy suggested for more economical use was to employ dilute aqueous solutions of fluorochemicals, since they were generally felt to offer better wetting of the stock. In spite of some improvement, dilute aqueous compositions of fluorochemicals nevertheless failed to provide a total solution to the problem. Such compositions had a tendency to flock, and therefore, a loss of potency upon standing resulted.

It has now been discovered that a group of fluorine-containing phosphate compositions when used in conjunction with a particular group of additives, either singly or in combination, are capable of inducing a cellulose swelling or wetting effect or a sequestration of metal ions when in contact with cellulosic fibers thereby providing enhanced fluorochemical activity. This is demonstrated by the fact that fluorochemical concentration of a bath at the beginning of a coating operation remains substantially undiminished at the time of completion. By employing the foregoing additives in an aqueous fluorochemical bath, the activity of the oleophobic ingredients is potentiated over corresponding compositions used in the absence of such additives. The treated stock is also more uniformly oleophobic, and therefore, all paper and paperboard stock, regardless of the type and source of pulp, method 25 of making, particular pigment or binder content, will now respond economically to fluorochemical application.

Accordingly, it is a principal object of the present invention to provide a series of novel fluorine-containing phosphate sizing compositions which can be employed 30 economically to virtually any type of cellulosic stock.

It is a further object of the instant invention to provide potentiated fluorochemical compositions having improved oil and grease repellent properties when applied to sized cellulosics.

35 A still further object is to provide a series of cellulosic materials which have been coated with improved oleophobic compositions.

These and other objects, features and advantages of 40 this invention will become apparent to those skilled in the art after a reading of the following more detailed description.

### PREFERRED EMBODIMENTS OF THE INVENTION

45 In accordance with the present invention, functional surface coating compositions are prepared by incorporating from 0.025 to about 2.0 percent by weight of an active fluorine-containing phosphate material with about 0.01 to about 20.0 percent by weight of nonfluorinated organic and inorganic wetting or swelling agents either alone or in combination with sequestering agents which function to complex and/or chelate metal ions. With the presence of a sufficient amount of the nonfluorine containing additive, fibers of a cellulosic substrate become more receptive to efficient fluorochemical distribution and deposition. The additive-potentiators include various sequestering agents, water miscible organic solvents, surfactants and alkalis, each serving to either complex, wet or swell fibers of a cellulosic substrate for more favorable fluorochemical application. Though satisfactorily used individually, the additives are preferably employed in combinations, such as a plurality of water miscible solvents, like mixtures consisting of an aliphatic alcohol and dioxane or tetrahydrofuran (THF) or a monohydric alcohol such as n-butanol with THF and a chelating agent, such as DEG (the sodium salt of diethanol glycine).

70 Fluorochemicals found specially adaptable for use in the subject-compositions are fluorine-containing linear, branched and cyclic structured phosphates consisting of



from commonly available, water soluble primary, secondary and tertiary amines which are inclusive only by way of example of organic amines, such as alkyl amines, alkanolamines, nitrogen containing heterocyclics, cyclic amines, polyamines, and the like. Alkyl amines may be primary, secondary or tertiary and may have alkyl groups having 1 to 6 carbon atoms. The alkyl portion of the amines may be straight chain or branched like methylamine, ethylamine, diethylamine, triethylamine, tripropylamine, diisobutylamine. Alkyl amines also encompass mixed amines such as N-ethyl-dipropylamine, N-ethyl-N-methyl propylamine, N,N-dimethyl butylamine, etc. Alkanolamines which form substituted ammonium salts with the taught compounds usually have from 1 to 3 hydroxyl groups and may also be primary, secondary, or tertiary amines. Examples of suitable alkanolamines are monoethanolamine, diethanolamine, triethanolamine, bis(2-hydroxypropyl) amine and pentanolamine and related compounds having 2 and 3 hydroxy groups and in the range of from 2 to 10 carbon atoms. Substituted ammonium salts also may be prepared from nitrogen-containing heterocyclic compounds including aromatic and non-aromatic types which may or may not be substituted, like imidazole, morpholine, piperidine and alkyl substituted heterocyclics having 1 to 6 carbon atoms like 2-ethyl imidazole. Cyclic amines and especially bicyclic compounds like triethylenediamine are useful salt forming agents. Suitable polyamines are ethylenediamine, 1,2-propanediamine, diethylene triamine, etc.

Preparation of the foregoing salts are described in co-pending patent application S.N. 236,978, filed Mar. 22, 1972. The fluorochemical compounds and salts disclosed therein and methods for their manufacture are hereby incorporated-by-reference into the present application.

Functional surface coating compositions will generally contain from about 0.025 to about 2.0 percent by weight of the fluorine-containing material, and most frequently, from about 0.05 to about 1.0 percent. However, more optimal quantities of fluorochemical will range from about 0.05 to about 0.5 percent by weight.

The non-fluorinated materials used in combination with the aforementioned fluorochemicals are mainly organic compounds providing wetting or swelling effect when in contact with cellulosic fibers. Inorganic compounds may also be used for enhanced oleophobic properties, for example, alkali metal hydroxides, carbonates and acids, such as boric acid and the like. In addition, certain of these non-fluorinated materials function as sequestering agents which form complexes when in contact with cations, such as those commonly found, for example, in clay and alum sizing. They also operate by sequestering or chelating these ions for more efficient deposition, orientation and distribution of the fluorochemical on the substrate. Particularly useful non-fluorinated materials falling within this definition are water-miscible organic solvents, chelating agents, non-ionic surfactants and alkali metal hydroxides.

A wide range of water-miscible organic solvents are recommended including readily available alcohols, such as methanol, ethanol, propanol, butanol, amyl alcohol and the like. The alcohols are preferably aliphatic, monohydric compounds having from about 1 to about 7 carbon atoms. Other available water miscible solvents include inter alia dimethylformamide (DMF), tetrahydrofuran (THF), dioxane, acetone, methyl ethyl ketone and the like. Generally, a cellulosic wetting amount of solvent or an amount sufficient to cause a swelling of cellulose fibers should be added to the fluorochemical. Excessive quantities of solvent are neither required nor recommended. More specifically, the water miscible organic solvents may be used in amounts from about 1 to about 20 percent, and more preferably, from about 4 to about 8 percent by weight.

It is also specially advantageous to employ combinations of such water miscible organic solvents with the fluorochemicals disclosed herein. For example, blended

5 admixtures of n-butanol and THF, DMF or dioxane are particularly effective when employed with the oleophobic fluorochemicals. N-amyl-alcohol can also be satisfactorily used in combination with DMF for enhanced oleophobicity. Other variations of organic solvent combinations too numerous to mention, provide acceptable results. However, in selecting a particular solvent or combination of solvents for use with the fluorochemical ingredient preferably they should be readily miscible in aqueous solutions. The proportional range of each solvent used in a given combination of solvents is not critical, however, the combined quantities employed in a coating composition will not ordinarily exceed those amounts set-forth above for homogeneous solvent containing compositions.

15 As previously mentioned, the sequestering agents operate by complexing or chelating cations commonly found in cellulosic sizing. For purposes of the present invention, sequestering agents are inclusive of complexing compounds, such as chelating agents which include both organic and inorganic materials capable of reacting with metallic ions to form complex molecules. Typical examples include compounds and salts, such as sodium tetraborate decahydrate, ammonium pentaborate, disodium octaborate tetrahydrate, sodium salt of diethanol glycine (DEG), sodium citrate, potassium citrate, the alkali metal salts of ethylenediaminetetraacetic acid, diethylenetriaminepentacetic acid-pentasodium salt, nitrilotriacetic acid disodium salt (monohydrate), N-hydroxyethyl ethylenediaminetriacetic acid (trisodium salt), oxalic acid, citric acid, boric acid and sodium hexametaphosphate, sodium acid pyrophosphate, monosodium phosphate, sodium carbonate, and the like. Ordinarily, all that is needed is a complexing amount or an amount sufficient to bind or sequester the metallic ions on the cellulose fibers. More particularly, sequestering agents of the present invention are used with fluorochemicals in an amount ranging from about 0.1 to about 2.0 percent by weight, and most advantageously, from 0.25 to about 0.75 percent by weight.

20 Enhanced oleophobic properties are also attainable using combinations of different sequestering agents or mixtures of sequestering agents and water miscible organic solvents. Representatives of this preferred combination, only by way of example include, n-butanol and diethylenetriaminepentacetic acid pentasodium, n-butanol and ethylenediaminetetraacetic acid disodium, diethanol glycine sodium salt, n-butanol and THF, sodium citrate and n-butanol, sodium hexametaphosphate and n-butanol, etc. Combinations, such as boric acid and sodium tetraborate decahydrate are but one example of potentiating combinations of chelate-sequestering compositions. Proportional amounts of each chelant, where a plurality of such materials are used, is not critical, however, the total quantity in compositions containing more than one of such agents or in blends with solvents should be from about 0.25 to about 0.75 percent by weight.

25 30 35 40 45 50 55 60 65 In addition to water soluble solvents and chelating agents, various surface active agents and alkali metal hydroxides like sodium and potassium hydroxides impart favorable properties in terms of enhanced oleophobic activity to cellulosic fibers. Various types, including anionic, cationic and amphoteric type surface active agents are satisfactory, however, non-ionic surfactants stand out as being specially preferred. Oleophobic properties of the fluorochemicals are further improved when such surfactants are employed with water miscible organic solvents.

Typical non-ionic types include a series of emulsifiers known as "Surfynols" which are ethylene oxide adducts of acetylenic glycols of the formula:



70 75 wherein  $\text{R}_1$  and  $\text{R}_4$  are alkyl radicals containing from 3

to 10 carbon atoms,  $R_2$  and  $R_3$  are selected from the group consisting of methyl and ethyl,  $x$  and  $y$  have a sum in the range of 3 to 60. Representative "Surfynols" include among others "Surfynol 440" which is the ethylene oxide adduct 2,4,7,9-tetramethyl-5-decyne-4,7-diol.

Nonionics also include the polyoxyethylene nonylphenyl ethers available under the trade name "Igepal." "Igepal CO-630" is a polyoxyethylene nonylphenyl ether having a cloud point of between 126° and 133° F. Other representative examples include esters of sulfon succinic acid, as for example, the sodium diethyl ester available under the trade name "Aerosol OT" or "Monowet MO-70-E" and the sodium diisobutyl ester sold under the names "Aerosol IB" and "Monowet MB-70." Other esters, such as di-tridecyl sodium, and di-hexyl sodium are well adaptable to the subject-compositions and are also commercially available through ordinary channels of commerce.

Surface-active agents are generally added to fluorochemicals in an amount sufficient to provide a wetting or swelling effect upon the cellulosic fibers, and more specifically, in an amount from about 0.01 to about 1.0 percent by weight. However, as in the case of chelating agents they are most advantageously used in combination with the water miscible organic solvents for more optimal performance of the fluorochemical. The ratio of surfactant to solvent should generally range from about 1:40 to about 1:400 and more preferably from about 1:40 to about 1:160.

The functional surface coating compositions of the instant invention are well adapted for application to virtually all types of cellulosic materials, such as paper and paperboard, sized and unsized stock prepared from sulphite, Kraft, soda, groundwood and other types of non-chemical and semichemical grades.

Although the aqueous compositions of the present invention can be applied to paper or paperboard, either on-machine or off-machine, most commonly they would be applied to at least one or perhaps both sides by means of an on-machine size press or at the calender stack. In these processes, the composition is sprayed, cascaded or transfer rolled onto the web, or the web is immersed in the size bath, and the excess size is then metered off by either a wire wound rod or by nip rolls or both.

The wet web then feeds through a circulating hot air oven, infrared bank or over a hot drum and/or hot calender to dry the treated paper at from 180° to 450° F., depending on the rate at which the web travels. The dried treated stock is roll wound or cut to size and stacked ready for use.

Where it is convenient to add a known quantity of the fluorochemical composition directly to the furnish at the beater or repulper, cationic retention aids, known in the art, are added thereto. The stock is then sheeted and dried as above.

In order to evaluate the effectiveness of the compositions of the present invention in terms of their ability to impart enhanced oleophobic properties to cellulosic materials and to demonstrate their superiority over conventional surface coating products, the following test procedure was adopted:

#### OIL PENETRATION TEST

##### Apparatus requirements:

1. A tube of any rigid material, 2.5 cm. (1 in.) ID and at least 2.5 cm. (1 in.) in height, the ends of which have been smoothed.
2. A pipet or medicine dropper, calibrated to deliver 1.1 ml.
3. Round-grained sand, Ottawa cement testing sand screened to pass a No. 20 and be retained on a No. 3 sieve.
4. Sheets of white coated and calendered 80 lb. book paper, 104 grams/m. exponent to, 70 lb. at least the same size as the test specimen, preferably much larger.
5. A stop watch or laboratory timer. The reagents, peanut

oil, nujol, liquid lard and corn oil are separately placed in bottles (100 ml. in each bottle) with 1.0 gram of an oil soluble red dye.

Each specimen is then placed on a sheet of book paper resting on a smooth flat surface. An end of the tube is placed on the specimen and 5 grams of sand is placed in the tube. The purpose of the tube is solely to insure a uniform area of the sand pile. Using the pipet or a medicine dropper, 1.1 ml. of the colored oil or greases were added to the sand, the tube is removed, and the timing device is started. The test proceeds for 72 hours at 60° C. or until the stain strikes through the treated paper and stains the book paper beneath it.

The following specific examples illustrate the compositions and processes of the instant invention and their improved oleophobic properties when applied to cellulosic substrates. It is to be understood, however, that these examples are for illustrative purposes only and do not purport to be wholly definitive as to conditions and scope.

#### EXAMPLE I

A size bath composition having the following ingredients was prepared:

|                                                                                                                   | Parts by weight |
|-------------------------------------------------------------------------------------------------------------------|-----------------|
| Water                                                                                                             | 78.5            |
| Sodium tetraborate decahydrate                                                                                    | 0.5             |
| n-Butanol                                                                                                         | 4.0             |
| THF                                                                                                               | 2.0             |
| 1% solution diethanolamine salts of mono, bis and pyroesters of 1,1 dihydropiperfluorocyclohexanemethyl phosphate | 15.0            |
|                                                                                                                   | 100.0           |

The ingredients were blended together in a vessel in the order shown until a homogeneous mixture resulted. The bath had 0.15% fluorochemical content.

(A) A sheet of 50 lb. southern kraft having 0.6% rosin/alum sized was completely immersed in the bath containing 0.15% fluorochemical phosphate (FC). After removal, it was padded to drain off excess fluid, dried for 15 minutes at 180° F. in a circulating hot air oven, and found to contain 0.19% active FC on the weight of paper. The dried fluorochemical treated sheet was tested in accordance with ASTM Standard Method F87-68 outlined above using peanut oil. Average creased peanut oil holdout was 23 hours at 60° C.

(B) For purposes of comparison, an aqueous bath was prepared with a 0.6% concentration of the same fluorochemical phosphate. However, no solvents or chelating agents were added. A sheet of 50 lb. southern kraft with 0.6% rosin/alum sized was immersed and dried in accordance with the method of part A and found to contain 0.46% active FC on the weight of paper. Using the same method of testing the average creased peanut oil holdout was less than 1/4 hour at 60° C.

Part (A) which compositions contain both FC and additives of the present invention and those of part (B) which contain no additives demonstrate that in spite of higher FC concentrations on weight of paper for the latter, more efficient deposition, orientation and distribution of FC can be achieved for more enhanced oil repellency with the former. The results are especially dramatic when taken in light of part (A) which had a bath concentration of only 0.15% FC, whereas part (B) composition had a FC bath concentration of 0.6%.

#### EXAMPLE II

A composition was prepared corresponding to that outlined in Example I (A), however, 0.5% diethanol glycine sodium salt was used in place of the sodium tetraborate decahydrate. Using 50# southern kraft (0.6% rosin/alum sized), creased holdout was increased to 50 hours at 60° C. for paper found to contain 0.16% active FC.

**9**  
**EXAMPLE III**

A sizing bath having the following ingredients was prepared:

|                                                                                                                                             | Parts by weight | 5  |
|---------------------------------------------------------------------------------------------------------------------------------------------|-----------------|----|
| Water                                                                                                                                       | 95.8            |    |
| n-Butanol                                                                                                                                   | 4.0             |    |
| [F(CF <sub>2</sub> ) <sub>7</sub> CH <sub>2</sub> O] <sub>2</sub> P(O)[OH <sub>2</sub> N(CH <sub>2</sub> CH <sub>2</sub> OH) <sub>2</sub> ] | 0.2             |    |
|                                                                                                                                             | 100.0           | 10 |

The above ingredients were combined and mixed in the order shown. A sheet of 50# southern kraft (0.6% rosin/alum sized) was entirely immersed in the composition, excess FC squeezed off and the sheet dried at 180° F. The average creased peanut oil holdout was 41 hours at 603 C. based upon 0.25% active fluorochemical on weight of paper. In comparison, when n-butanol is excluded from the composition, 0.31% active FC is picked up and average creased peanut oil holdout is less than 1/4 hour at 60° C.

Compositions corresponding to those in Example III were also prepared, however, the quantity of fluorochemical was gradually increased. Results are shown in the table below.

TABLE I

| Percent fluorochemical in bath | Percent fluorochemical on weight of paper | Creased peanut oil holdout (hours at 60° C.) |
|--------------------------------|-------------------------------------------|----------------------------------------------|
| 0.4.....                       | 0.43                                      | 72+                                          |
| 0.6.....                       | 0.54                                      | 72+                                          |
| 0.8.....                       | 0.75                                      | 72+                                          |

Table I demonstrates the oleophobicity imparted to celullosic material by a given composition is not directly proportional to the concentration of fluorochemical present. Optimal oil repellency properties can be achieved with compositions having lower concentrations of fluorochemical, provided, a nonfluorinated additive, is included, e.g. water-miscible organic solvent (n-butanol).

To further demonstrate the effect of the additives, aqueous compositions of the same fluorochemical of Example III were prepared without non-fluorinated organic or inorganic additives, which is inclusive of water-miscible organic solvents, sequestering agents or surfactants. The results are found in the table below.

TABLE II

| Percent fluorochemical in bath | Percent fluorochemical on weight of paper | Creased peanut oil holdout (hours at 60° C.) |
|--------------------------------|-------------------------------------------|----------------------------------------------|
| 0.2.....                       | 0.11                                      | <0.25                                        |
| 0.4.....                       | 0.24                                      | <0.25                                        |
| 0.6.....                       | 0.31                                      | <0.25                                        |
| 0.8.....                       | 0.33                                      | <0.25                                        |

Table II provides evidence that conventional aqueous fluorochemical coating compositions applied to sized stock, regardless of the fluorochemical concentration, does not impart acceptable oil repellency properties to such cellulosics. In contradistinction, the compositions of Examples I(A), II and III all prepared with the non-fluorinated additives of the subject invention for improved deposition, orientation and distribution of the FC on cellulose stock, provided a fluorochemical on weight of paper at a percentage well within the range shown in Table II, however, the average creased peanut oil holdout ranged from 23 to 50 hours rather than the 1/4 hour or less holdouts of Table II.

**10**  
**EXAMPLE IV**

|                                                                                                                  | Parts by weight |
|------------------------------------------------------------------------------------------------------------------|-----------------|
| Water                                                                                                            | 79.5            |
| Diethanol glycine sodium salt                                                                                    | 0.5             |
| 1% solution diethanolamine salts of mono, bis and pyroesters of 1,1 dihydroperfluorocyclohexane methyl phosphate | 20.0            |
|                                                                                                                  | 100.0           |

The ingredients were mixed in the order shown until a homogeneous solution was prepared. A sheet of 41# Reg. waterleaf (bleached kraft) was immersed completely into the solution having a fluorochemical concentration of 0.2%. Upon removal, excess fluid was allowed to drain off and the sheet dried at 180° F. in a circulating hot air oven. The sheet was tested for oil repellency according to the above method. The percent fluorochemical on weight of paper was 0.23 and the creased peanut oil holdout was 72+ hours at 60° C.

A control solution containing no diethanol glycine sodium salt had a creased peanut oil holdout of less than 0.25 hour.

25

## EXAMPLE V

|                                                                                                                  | Parts by weight |
|------------------------------------------------------------------------------------------------------------------|-----------------|
| Water                                                                                                            | 65.95           |
| n-Butanol                                                                                                        | 4.00            |
| Surfynol 61 (3,5-dimethyl-1-hexyn-3-ol)                                                                          | 0.05            |
| 1% solution diethanolamine salts of mono, bis and pyroesters of 1,1 dihydroperfluorocyclohexane methyl phosphate | 40.0            |
|                                                                                                                  | 100.0           |

A composition was prepared by admixing the above ingredients in the order shown until a homogeneous solution having 0.4% fluorochemicals resulted. In order to determine its oleophobic properties a sheet of 50 lb. natural southern kraft (0.6% rosin/alum sized) was immersed, drained and oven dried at 180° F. The percent fluorochemical on weight of paper was 0.70% and the creased peanut oil holdout was 25 hours at 60° C.

As a control, an aqueous composition was also prepared with 0.4% active fluorochemical in the bath along with 4% n-butanol and no surfactant. The percent fluorochemical on weight of paper was 0.72 and the creased peanut oil holdout was 7 hours at 60° C.

While the invention has been described in conjunction with specific examples thereof, they are illustrative only. Accordingly, many alternatives, modifications and variations will be apparent to those skilled in the art in light of the foregoing description, and it is therefore intended to embrace all such alternatives, modifications and variations as to fall within the spirit and broad scope of the appended claims.

I claim:

1. A functional surface coating composition consisting essentially of (1) from about 0.01 to about 20.0 percent by weight of nonfluorinated material selected from mixtures consisting of alkali metal hydroxides and carbonates, dimethylformamide and tetrahydrofuran and (2) from about 0.025 to about 2.0 percent by weight of a fluorine containing phosphate material consisting essentially of polyfluoroalkyl and cycloalkyl phosphates of the formula (R<sub>2</sub>L)<sub>3-y</sub>Z where:

R<sub>2</sub> is:

R<sup>2</sup>(CF<sub>3</sub>)<sub>a</sub>—, where R<sub>2</sub> is H and a is an integer of from 1 to 20;

(CF<sub>3</sub>)<sub>2</sub>CR<sub>3</sub>(CF<sub>3</sub>)<sub>b</sub>—, where R<sub>3</sub> is F or H and b is 0 and R<sub>3</sub> is F when b is an integer of from 1 to 18;

or R<sub>4</sub>(c-C<sub>6</sub>F<sub>10</sub>)—, where R<sub>4</sub> is F or C<sub>n</sub>F<sub>20+1</sub> and n is an

70

75

## 11

integer of from 1 to 4 and where c- designates an alicyclic structure;  
L is:



where  $R_5$  is an alkyl group having 1 to 10 carbon atoms; or  $(CH_2)_nO-$ , where  $n$  is the integer 1 or 2; y is an integer of 1 or 2, and

Z is:

$-P(L)(OM)x$  where  $x$  is an integer of 1, 2 or mixtures thereof and M is a water-solubilizing cation of the group consisting of alkali metal, ammonium and substituted ammonium when  $x$  is 1, and each M is independently selected from the group consisting of hydrogen, alkali metal, ammonium and substituted ammonium when  $x$  is 2.

2. The composition of claim 1 wherein the fluorine containing phosphate is



3. The composition of claim 1 wherein the fluorine containing phosphate is



4. The composition of claim 1 wherein the fluorine containing phosphate is



5. The composition of claim 1 wherein the fluorine containing phosphate is



6. The composition of claim 1 wherein the solvent and chelating agents comprise a mixture of n-butanol, diethanol glycine sodium salt and tetrahydrofuran.

7. The composition of claim 1 wherein the solvents comprise a mixture of n-butanol and tetrahydrofuran.

8. A functional surface coating composition comprising (1) from about 0.01 to about 20.0 percent by weight of a nonfluorinated material selected from the group consisting of alkali metal hydroxides and carbonates, chelating agents, nonionic, anionic and cationic surfactants, alcohols containing 1-7 carbon atoms, dimethylformamide, tetrahydrofuran, dioxane, acetone, methyl ethyl ketone and mixtures thereof and (2) from about 0.025 to about 2.0 percent by weight of a polyfluorocyclohexyl phosphate comprising a mixture of mono, bis and pyroesters of the formula:



and



wherein  $K_f$  is fluorine or a  $C_1$  to  $C_4$  perfluoroalkyl group substituted on the 2, 3 or 4 position of the cyclohexane ring,  $n$  is an integer of from 1 to 4,  $a$  is an integer of from 1 to 2 and X in each occurrence is independently selected from chlorine or any member of OM where M is a water-solubilizing cation of the group consisting of hydrogen, alkali metal, ammonium and substituted ammonium.

9. The composition of claim 8 wherein the polyfluorocyclohexyl phosphate comprises mixtures of compounds in which X is OM, M is hydrogen,  $a$  is 1,  $n$  is 2 and  $K_f$  is F.

10. The composition of claim 8 wherein the polyfluorocyclohexyl phosphate comprises mixtures of compounds in which X is OM, M is hydrogen,  $a$  is 1,  $n$  is 1 and  $K_f$  is F.

## 12

11. The composition of claim 8 wherein the polyfluorocyclohexyl phosphate comprises mixtures of compounds in which X is Cl,  $a$  is 1,  $n$  is 1 and  $K_f$  is F.

12. The composition of claim 8 wherein the polyfluorocyclohexyl phosphate comprises mixtures of compounds in which X is Cl,  $a$  is 2,  $n$  is 1 and  $K_f$  is F.

13. The composition of claim 8 wherein the polyfluorocyclohexyl phosphate comprises mixtures of compounds in which X is OM, M is diethanol ammonium,  $a$  is 2,  $n$  is 4 and  $K_f$  is F.

14. The composition of claim 8 wherein the polyfluorocyclohexyl phosphate comprises mixtures of compounds in which X is OM, M is diethanol ammonium,  $a$  is 1,  $n$  is 1 and  $K_f$  is F.

15. The composition of claim 8 wherein the polyfluorocyclohexyl phosphate comprises mixtures of compounds in which X is OM, M is diethanol ammonium,  $a$  is 1 and 2,  $n$  is 1 and  $K_f$  is F.

16. A functional surface coating composition comprising (1) from about 0.01 to about 20.0 percent by weight of water miscible organic solvents and sequestering agents selected from the group consisting essentially of n-butanol, tetrahydrofuran, dioxane, diethanol glycine sodium salt, sodium tetraborate decahydrate, disodium octaborate tetrahydrate and mixtures thereof and (2) from about 0.025 to about 2.0 percent by weight of a polyfluorocyclohexyl phosphate comprising a mixture of mono, bis and pyroesters of the formulas:



and



wherein  $K_f$  is fluorine or a  $C_1$  to  $C_4$  perfluoroalkyl group substituted on the 2, 3 or 4 position of the cyclohexane ring,  $n$  is an integer of from 1 to 4,  $a$  is an integer of from 1 to 2 and X in each occurrence is independently selected from chlorine or any member of OM where M is a water-solubilizing cation of the group consisting of hydrogen, alkali metal, ammonium and substituted ammonium.

17. The composition of claim 16 wherein the solvents comprise a mixture of n-butanol and tetrahydrofuran.

18. The composition of claim 16 wherein the solvents comprise a mixture of n-butanol and dioxane.

19. The composition of claim 16 wherein the solvent and complexing agents comprise a mixture of n-butanol and diethanol glycine sodium salt.

20. The composition of claim 19 including tetrahydrofuran.

21. The composition of claim 16 wherein the solvent and complexing agents comprise a mixture of n-butanol and sodium tetraborate decahydrate.

22. The composition of claim 16 wherein the solvent and complexing agents comprise a mixture of n-butanol and disodium octaborate tetrahydrate.

60

## References Cited

## UNITED STATES PATENTS

|           |        |          |            |
|-----------|--------|----------|------------|
| 3,664,987 | 5/1972 | Moyer    | 260-29.6 H |
| 2,597,702 | 5/1952 | Benning  | 260-924    |
| 3,245,816 | 4/1966 | Schwaibe | 106-213    |
| 3,039,886 | 6/1962 | Masley   | 106-214    |
| 3,736,164 | 5/1973 | Uffner   | 106-213    |

## OTHER REFERENCES

70 Surface Active Agents—Schwartz, 1949.

THEODORE MORRIS, Primary Examiner

U.S. Cl. X.R.

UNITED STATES PATENT OFFICE  
CERTIFICATE OF CORRECTION

Patent No. 3,810,772 Dated May 14, 1974

Inventor(s) Melville W. Uffner

It is certified that error appears in the above-identified patent and that said Letters Patent are hereby corrected as shown below:

In the Specification:

Column 4, line 57, within the formula, after "C<sub>6</sub>", "H<sub>11</sub>" should be--F<sub>11</sub>--

Column 9, line 17, "603C" should be--60°C--

In the Claims: . . .

Claim 1 - Column 10, line 75, within the formula, "F<sub>20</sub>" should be--F<sub>2n</sub>--

Claim 2 - Column 11, line 24, in the formula, before "CF<sub>3</sub>" and after "[" insert--F--

Claim 5 - Column 11, line 35, "OH<sub>2</sub>" should be--CH<sub>2</sub>--

Signed and Sealed this  
twenty-seventh Day of April 1976

[SEAL]

Attest:

RUTH C. MASON  
Attesting Officer

C. MARSHALL DANN  
Commissioner of Patents and Trademarks